

1,386,277

R. P. PERRY,  
BUILDING FELT OR CONSTRUCTION MATERIAL,  
APPLICATION FILED OCT. 8, 1918.

Patented Aug. 2, 1921.



INVENTOR  
*Ray P. Perry*  
BY  
*Chas. W. Mortimer,*  
ATTORNEY

# UNITED STATES PATENT OFFICE.

RAY P. PERRY, OF UPPER MONTCLAIR, NEW JERSEY, ASSIGNOR TO THE BARRETT COMPANY, A CORPORATION OF NEW JERSEY.

## BUILDING-FELT OR CONSTRUCTION MATERIAL.

1,386,277.

Specification of Letters Patent.

Patented Aug. 2, 1921.

Application filed October 8, 1918. Serial No. 257,396.

To all whom it may concern:

Be it known that I, RAY P. PERRY, a citizen of the United States, residing at Upper Montclair, in the county of Essex and State of New Jersey, have invented certain new and useful Improvements in Building-Felt or Construction Materials, of which the following is a specification.

This invention relates to a new and useful building felt or construction material. It relates more specifically to felt which is made of fibrous material, or even paper stock fibers, having distributed therethrough comminuted waterproofing material in the form of shot or substantially spherical particles, or particles which are not extended greatly in any direction, but which are of appreciable size as contradistinguished to dust or powder.

It has been found that when particles of waterproofing material in the form of powder or dust is introduced into the paper or felt during the formation of the sheets on an ordinary paper-making machine having a foraminous cylinder, the sheets are not very porous, but the fibers are closely knit with the fine particles of waterproofing material filling, to a considerable extent, whatever interstices there may have been between the fibers, thus rendering the sheets incapable of readily absorbing a large amount of liquid waterproofing material. When waterproofing material in the form of filaments is introduced into the sheets in a similar manner the sheets are rendered more porous, but if the filaments are made of material that is brittle when cold, some of them will be broken into short pieces as a result of handling and bending the sheets after they are formed.

By this present invention the sheets have distributed therethrough particles of waterproofing material which are solid at ordinary temperatures and which are not considerably lengthened or extended in any direction. Preferably, the particles are in the form of shot or globules and are made of pitch or other bituminous material, though it is to be understood that the invention is not restricted to these particular shapes or materials, since oblong or spheroidal or other shapes which will not readily be broken upon bending the sheets may be used, and the materials may be rosin, wax, shellac, tallow or other waterproofing material which is solid

when cold. The size of the particles may vary from those having a dimension as great as one sixteenth of an inch down to those just large enough to be caught on a hundred mesh screen. The preferable sizes are those which will pass through a thirty mesh screen but will not pass through a hundred mesh screen. The porosity of the sheets will vary, depending somewhat upon the size and number of the particles distributed therethrough.

The invention will be readily understood from the accompanying drawing which is a side view of a paper-making machine, partly in section.

In this view reference character T represents a tank having a foraminous cylinder C therein upon which is formed the usual layer 2 of paper or felt which is picked up by means of the "wet blanket" 3 passing around the rolls 4 and 4'. The sheet passes along the suction box 5 where a portion of the water is removed and then under the squeeze roll 6 where more of the water is pressed out, after which it passes over the hot drying rolls 8.

In operation the usual paper or felt-making stock is introduced into the tank T together with the particles of solid waterproofing material, which become incorporated into the sheet 2 upon the cylinder C and form a part of this sheet. These particles being round, prevent the fibers from knitting or matting as closely as they otherwise would, thus making the sheet more porous and better adapted for absorbing liquid waterproofing material during the subsequent saturating operation whenever such an operation is desirable, as well as permitting ready drying or evaporation of the moisture during the drying operation. While any desired proportions of the ingredients used in making the sheet may be employed, I prefer to use between 10% and 90% by weight of waterproofing material the remainder consisting of paper or felt stock.

It is obvious that the drying may be done by air instead of hot cylinders, and that the saturation of the sheets with liquid waterproofing material may be accomplished, for example, by passing the sheets through a bath of the saturant.

The sheets produced in accordance with this invention are very porous and flexible;

they are not seriously impaired by repeated bending or flexing; they will readily absorb a large amount of waterproofing material; they are easily dried; they contain 5 a considerable proportion of waterproofing material in the form of solid particles even before any saturating operation with liquid waterproofing material takes place.

Claims:

- 10 1. As an article of manufacture, a sheet of porous, flexible building felt containing rounded particles of waterproofing material too large to pass through a hundred mesh screen.
- 15 2. As an article of manufacture, a sheet of porous, flexible building felt containing waterproofing material in the form of shot of appreciable size, and fibrous material.

3. In an article of manufacture, a sheet of porous, flexible building felt containing 20 bituminous material in the form of shot of appreciable size, and fibrous material.

4. As an article of manufacture, a sheet of porous, flexible building felt containing pitch in the form of shot of appreciable 25 size, and fibrous material.

5. As an article of manufacture, a sheet of porous, flexible building felt consisting of between 10% and 90% of waterproofing material in the form of rounded particles 30 in size which will pass through a thirty mesh screen but will be caught on a hundred mesh screen, and fibrous material.

In testimony whereof I affix my signature.

RAY P. PERRY.